

## UNITED STATES PATENT OFFICE

2,270,191

## MAGNESIUM BASE ALLOY

John C. McDonald, Midland, Mich., assignor to  
 The Dow Chemical Company, Midland, Mich.,  
 a corporation of Michigan

No Drawing. Application October 4, 1940,  
 Serial No. 359,683

3 Claims. (Cl. 75—168)

The invention relates to a magnesium base alloy. It more particularly concerns an alloy of this nature having improved physical properties, such as high yield and tensile strengths.

Commercially pure magnesium has been used only in a limited way as a structural material because of its relatively low strength, although its light weight is a highly desirable characteristic.

It is, therefore, the principal object of the invention to provide a magnesium base alloy which possesses the light weight characteristic of magnesium and at the same time is endowed with superior strength characteristics.

Other objects and advantages will be apparent as the description of the invention proceeds.

My invention resides in the discovery that a magnesium base alloy containing from 0.01 to 4 per cent of platinum, the balance being magnesium, possesses the aforementioned properties of high tensile and yield strengths. The term "magnesium" used herein and in the appended claims is intended to include magnesium containing the ordinary impurities that are found in commercially pure metal, such as traces of nickel, iron, copper, and silicon. While the properties of high yield and tensile strengths are manifest over the entire range of composition indicated, I have found that in general the preferred combination of properties is found in those alloys containing from 0.1 to 2.5 per cent of platinum. A preferred composition having exceptionally high yield and tensile strengths is one containing about 1 per cent of platinum.

The following table, listing some of the properties of rolled sheet metal made from my new binary alloy and comparing these properties with those of magnesium, illustrates the improvement in yield strength and tensile strength of my new alloy over that of magnesium. The magnesium used in preparing the new alloy and for the purposes of comparison was obtained by subliming commercial magnesium.

Table

| Nominal composition in percent<br>(magnesium—<br>remainder—<br>Pt) | Annealed                             |                                        | Cold rolled                          |                                        |
|--------------------------------------------------------------------|--------------------------------------|----------------------------------------|--------------------------------------|----------------------------------------|
|                                                                    | Yield<br>strength in<br>lbs./sq. in. | Tensile<br>strength in<br>lbs./sq. in. | Yield<br>strength in<br>lbs./sq. in. | Tensile<br>strength in<br>lbs./sq. in. |
| 0.09                                                               | 7,000                                | 26,000                                 | 14,000                               | 25,000                                 |
| 0.33                                                               | 15,000                               | 31,000                                 | 19,000                               | 26,000                                 |
| 1.15                                                               | 16,000                               | 32,000                                 | 18,000                               | 29,000                                 |
|                                                                    | 18,000                               | 33,000                                 | 21,000                               | 33,000                                 |

The properties set forth above under the term

"annealed" were obtained by first rolling the specimens at a temperature of from 650° to 750° F. and thereafter annealing them at various temperatures of from 400° to 800° F. The properties selected for the table were those of the annealed specimens which exhibited the maximum elongation. The properties set forth under the term "cold rolled" were obtained by subjecting the specimens which had been first hot rolled at a temperature of from 650° to 700° F. to additional rolling in the cold state. The properties selected for the table were those of the cold rolled specimens which showed the greatest yield strength while having an elongation of at least 1 per cent in 2 inches.

A comparison of the properties listed in the above table shows that the yield strength and tensile strength of my new alloy are markedly superior to those of magnesium in both the annealed and the cold rolled state. The improvement shown in the above example is exhibited throughout the range of the alloying ingredient indicated.

The new alloy will be found to be most useful in making large castings, forgings, and the like where light weight coupled with high strength is desirable.

The new alloy may be prepared in any of the ways usually employed for alloying metals with magnesium, such as by adding the platinum to a bath of molten magnesium, which is preferably protected from oxidation by suitable flux.

I claim:

1. A magnesium base alloy containing from 0.01 to 4 per cent of platinum and characterized by a substantial improvement in at least one of the properties ductility, yield strength, and tensile strength as compared to magnesium without the platinum.

2. A magnesium base alloy containing from 0.01 to 4 per cent of platinum, the balance being magnesium.

3. A magnesium base alloy containing from 0.1 to 2.5 per cent of platinum, the balance being magnesium.

JOHN C. McDONALD.